

W. H. THOSS.  
FIRE PLATING IRON.

No. 25,291.

Patented Aug. 30, 1859.



W. H. Thoss  
Inventor

# UNITED STATES PATENT OFFICE.

WILLIAM H. THOSS, OF SAN FRANCISCO, CALIFORNIA.

## IMPROVEMENT IN FIREPLATING IRON.

Specification forming part of Letters Patent No. 25,291, dated August 30, 1859.

*To all whom it may concern:*

Be it known that I, WILLIAM H. THOSS, of the city and county of San Francisco, State of California, have invented and discovered a process or mode of fireplating iron in all its shapes and forms with copper, pure and alloyed, to be used in all mechanical, commercial, and mining purposes, and have invented and designed a furnace to be used in doing same; and I do hereby declare that the following is a full and exact description thereof, reference being had to the accompanying drawings, and to the letters of reference marked thereon.

The nature of my discovery and invention consists in plating with copper (pure and alloyed) by fire process iron in its various shapes—such as sheet-iron bars, flat and round, bolts, spikes, and nails, and all other forms—varying the shape or form of basin in the melting-furnace to suit the shape or form of the piece of iron to be plated.

The following is the process and apparatus required for plating sheet-iron, the same principle being applied to all other forms of iron, only varying the apparatus of tanks and metal-basin in furnace in size and shape, adhering to the principle of construction and draft obtained in furnace.

I make use of three tanks or vats, in which is placed the following: No. 1, a tank of diluted sulphuric acid; No. 2, a tank of clean water; No. 3, a tank of borax in solution; No. 4, melting-furnace for the copper, a plan of which is hereunto annexed.

I heat the water in borax-tank to or near a boiling heat to assist in dissolving the borax, and as soon as dissolved let it cool off, being then ready for use.

When I desire to prepare iron for plating, I bring the acid-vat near a boiling-point and place the sheets of iron in it for a sufficient length of time to bite or eat off the scale formed on surface of iron, and I then give them a good scouring with sand to assist in cleaning them, after which they are washed off in tank No. 2 (of clean water) and then thrown into the borax-vat No. 3, from which, after proper time, they are taken and placed in a warm room to dry off without being allowed to rust. When the sheets or whatever form the iron may be in is thus prepared it is ready to be dipped into the molten copper.

When the copper in basin or furnace has been brought to the proper degree of heat and fluid state, the sheet of iron is from one side run into the basin of copper and shoved through, being received at opposite side and drawn out, having received the coat of copper in its passage through the basin of metal, and is ready to be cleaned for whatever use it is to be put to.

I will now proceed to describe the construction and design of furnace, having reference to drawings hereunto annexed.

No. 1 presents full exterior side view of furnace. No. 2 presents full exterior end view of furnace. No. 3 presents side sectional view of interior. No. 4 presents end sectional view of interior. No. 5 presents ground or base plan of structure, showing system of draft-holes and ash-pits.

I construct the furnace of oval shape, main body being of common red bricks and interior of fire-surface of fire-bricks or other fire-resisting material.

View No. 1: A represents draft-hole, ash-pit, and grate-bars shown; B, opening for plates to be run through the metal in basin; C, chimney or flue.

View No. 2: A represents draft-hole, ash-pit, and grate-bars; B, opening for supplying fuel, closed by an iron door.

View No. 3, of furnace split lengthwise: A represents draft-holes and ash-pits terminating at pillar C; B, grate-bars; C C C C C, pillar on which basin-rest is constructed, of fire-brick or other fire-resisting material; D, basin for metal, of same material; E, fire-space and space of arch over basin, which draws the flame and heat to one common center and covers the basin, thereby producing the requisite heat on top of basin; F, opening for supply fuel; G, flue or chimney.

View No. 4, furnace split endwise: The same letters refer to same parts as described in No. 3, with exception that F shows the openings at both sides at which the sheets of iron are introduced into the basin of metal at one side and drawn out at the other.

View No. 5, ground or base of furnace: A A A represent the four draft-holes and ash-pits. The construction of these four drafts in correspondence with the arch and flue in the center produces an equally-distributed heat around the basin under and over, which

gives the requisite heat for melting the metal with the openings and surface required to allow of the immersing of large sheets of iron; B, main body of brick-work; C, base of pillar supporting basin.

I am aware that prior to my said invention it has been proposed to fireplate iron with copper or the alloys of copper by first cleansing the surface of the iron in dilute acids, and, after drying, coating it with clay by immersing it in a mixture of clay and water, and then drying by a brisk fire, and then dipping it in melted copper in an open heated crucible, and therefore I do not wish to be understood as making claim to any such mode of procedure; nor, broadly, to the process of fireplating iron with copper by dipping the iron in molten copper; but

What I do claim as my invention, and desire to secure by Letters Patent, is—

Preparing the iron, after it has been cleansed with dilute acid, by immersion in a solution of borax, and after being dried passing it through the molten copper maintained at the required heat in a furnace constructed, substantially as herein described, with a roof to concentrate the heat over the basin of molten copper and with an aperture at one side to insert the iron to be plated, and a corresponding one on the opposite side to receive the iron as it is drawn from the copper plated, substantially as described, and for the purpose specified.

San Francisco, June 18, 1858.

W. H. THOSS.

Witnesses:

GEO. A. VAN BOKKELAN,  
WM. HAYES.